

# United States Patent Office

2,970,883

Patented Feb. 7, 1961

1

2,970,883

## MANUFACTURE OF VISCOSE RAYON

Aart Buurman, Velp, and Robbert Aldert Vroom and Pieter Coenraad Limburg, Arnhem, Netherlands, assignors to American Enka Corporation, Enka, N.C., a corporation of Delaware

No Drawing. Filed Dec. 24, 1956, Ser. No. 630,033

Claims priority, application Netherlands Jan. 16, 1956

8 Claims. (Cl. 18—54)

This invention relates to the manufacture of viscose rayon and more particularly to an improvement in the viscose process and improved cellulosic products produced therefrom.

In the viscose rayon industry today it is rather common practice in the production of yarns having very high tenacity to retard or modify the regeneration process of the cellulose. This is done by adding certain chemicals either to the acid spinbath or to cellulose base material at some stage in the production of viscose prior to extrusion which retard the regenerating of the cellulose. These chemicals have become known in the art as viscose modifiers.

By using a modifier it is possible to produce yarns having a very high strength and improved soil and abrasion resistance. Furthermore, the cross-section of the modified yarns reveals filaments which have substantially all skin and very little, if any, sensitive core and which have peripheries of notably reduced crenulations. Also, the modified yarns are characterized by greater toughness, greater fatigue resistance and reduced gel swelling.

Although the general idea of chemically modifying the coagulating-regeneration process in the production of viscose rayon is old, the problem of selecting the most desirable modifying agent is by no means simple. Some of the considerations given in selecting a modifier include consideration of price, ease in preparation, commercial availability, solubility in viscose and solubility in spinbath. But the most important consideration to be given is the effect it has on the yarn produced. For example, one type of modifier may influence the production of an all skin yarn which may be very brittle. In other words, the flex-life of the yarn may be sacrificed for a gain in tenacity. Therefore, a need for a modifier which is effective in producing a modified yarn having the most optimum balance of the possible modifying effects exists in the industry today.

In U.S. Patent No. 2,593,466 it was disclosed that by incorporating into the viscose at any stage of its preparation about 0.01 to 0.2% by weight of a product formed from the reaction of at least about 12 moles of alkylene oxide with 1 mole of a primary or secondary aliphatic amine or mixture thereof, the amines containing from 6 to 18 carbon atoms, certain spinning difficulties could be overcome. However, viscose modification at the time was not known in the art, and the amine was used for an entirely different purpose, namely, to prevent clogging of the spinneret orifices.

One of the most promising class of modifiers is a type of organic compound which contains a polyoxyethylene structure. Many of these compounds of this type have been suggested. Such substances include castor oil condensed with alkylene oxide, residual oil of sulfitic liquors from wood pulp condensed with alkylene oxide, urea condensed with alkylene oxide and phenol condensed with alkylene oxide.

In another known process, as disclosed in British Patent No. 741,728, a viscose modifier with the general formula,

2

$RO-(C_2H_4O)_n-R_1$ , in which R represents an alkyl or an aryl radical and  $R_1$  represents an alkyl radical, an aryl radical or hydrogen and  $n$  is a number of four or less is suggested as an agent to modify the formation of rayon so that threads having a lower swelling value and a greater skin area as compared with filamentous products produced from unmodified viscose may be formed.

Furthermore, it has previously been found that threads with an increased skin character and a lower swelling value may be manufactured from viscose when the regeneration of the cellulose is carried out in the presence of a polymer, copolymer or block polymer of epoxy-alkanes or their substitution products.

However, a notable disadvantage connected with the known polyoxyalkylene type of viscose modifiers is that optimum results can only be secured by strictly controlling the number of alkylene oxide units present in the modifier which is indeed expensive and difficult to do.

An object of the present invention is to provide a process for the manufacture of regenerated cellulosic products having improved properties such as high tenacity and high fatigue resistance suitable for use in high tenacity industrial cords and better textile fabrics.

Another object of this invention is to provide a process for regenerating cellulose filaments, films and the like which are modified in a spinbath.

A further object of this invention is to provide a viscose modifier which exerts an optimum modifying effect upon the coagulation and regeneration of cellulose in a spinbath.

Still another object is to provide a cellulosic material having improved properties.

It is further an object of this invention to provide both a viscose solution and viscose spinbath containing a viscose modifier whereby a product of enhanced properties is obtained.

A general advance in the art and other objects which will appear herein are also contemplated.

In accordance with the present invention, viscose of desired ripeness is extruded through a spinneret into a zinc-containing acid spinbath in the presence of an organic compound containing alkylene oxide units which exert a decided modifying effect on the coagulation and regeneration process occurring in the bath. By incorporating in the spinbath or in the viscose at any stage of its preparation or both from 0.01%—1.0% by weight of one or more of the compound comprising an organic radical ( $R_1$ ) with not more than 7 carbon atoms bound to one or more  $-(RO)_n-R-R_2$  radicals, wherein R represents an aliphatic radical with two or more carbon atoms and  $R_2$  represents an organic radical with not more than 7 carbon atoms or a hydroxyl group and wherein  $n$  represents a whole number of at least 10, the regeneration-coagulation process is modified in a remarkable manner to produce regenerated cellulosic filaments, yarns, films and the like exhibiting improved properties. It is preferred that the ratio of the acid content in the spinbath to the alkali content in the viscose be about 1.3 to 0.8.

The organic radicals  $R_1$  and  $R_2$  may consist of alkoxy, aryloxy, thio-alcohol, thiophenol, acyloxy and acyl imino radicals. Furthermore, compounds may be used which are produced by the condensation of alkylene oxide with aldehydes, ketones, esters and isocyanates. However, the limiting condition is that the number of carbon atoms in said organic radicals should not exceed 7 because it has been found that with a larger number of carbon atoms the modifying effect of the polyalkylene oxide structure notably decreases.

One of the advantages of the present invention is that the number of alkylene oxide units is not critical. The modifier according to the present invention may contain

preferably more than 10 alkylene oxide units with no definite restriction on the upper limit. Compounds containing 100 and more units have been found to be effective as a modifier.

Another disadvantage connected with the use of known polyoxyalkylene type of viscose modifier is that there is a tendency of the viscose containing the modifier to foam during the deaeration of the viscose. This foam is highly undesirable since it impedes the deaeration process and may foam to such an extent that viscose may enter the vacuum conduits which make it necessary to limit the amount of viscose which may be deaerated in a tank of given size. Also, the foam is difficult to destroy. If foamy viscose is spun, the yarn quality is very poor and filamentary breaks occur quite frequently in the spinning process.

An unexpected advantage of the modifiers according to the present invention is that there is no foaming problem present during the deaeration of the viscose when the modifier has been incorporated in the viscose prior to deaeration.

Examples of compounds in their structural formulae which have been found particularly useful are:



Of the foregoing compounds the reaction products of alkylene oxides with aldehydes and ketones may be especially attractive because they are stable in the viscose but are decomposed by acid. Thus, said compounds will be decomposed and will not build up in the spinbath to an undesirable amount.

Generally the best yarn is obtained when the spinbath contains at least 3% by weight of a zinc salt and the acid content in the spinbath is not over 7% by weight. Besides the acid and the zinc salt, the spinbath may also contain other usual substances such as sodium sulfate or magnesium sulfate. The quality of the yarn may be further improved if the spun yarn is treated in the conventional two bath system in which the yarn is stretched

about 100% in the second bath. The stretching gives the threads a low swelling value.

The following examples illustrate methods carried out in accordance with the invention and are not to be construed as limitative.

#### Example I

A viscose with a cellulose content of 7.3% and an alkali content of 5.5% and containing 0.1% of a compound with the formula,



15 was extruded through a spinneret in the usual manner into a primary spinbath. The viscose had a xanthate ratio of 0.49, a viscosity of 45 sec. by the falling ball test and a ripeness of 15° Hottenroth. The spinbath contained 5.6% H2SO4, 16.4% Na2SO4 and 5.0% ZnSO4 and had a temperature of 62° C. For the purpose of increasing the spinning speed, the threads were directed in the primary spinbath through a two-diameter tube spinning device as described in the copending application, Serial No. 556,256, now Patent No. 2,908,937, assigned to the same assignee as the present application. The yarn was then directed in the usual manner into a second bath having a temperature of 90° C. and having an acid concentration of about one-twentieth of the first spinbath. During the travel in the second bath the yarn 20 was stretched 105% with the final draw-off speed being 80 meters per minute. The yarn was aftertreated in the usual way.

The two-diameter tube comprised a tube of two different diameters, the inlet opening of which having a flat trumpet-shaped flange disposed 2 cm. from and coaxially with the spinneret. The diameter of the tube portion closer to the spinneret was 21.5 mm. with the second portion being 26 mm. The length of the narrow and the wide tube portions were 40 and 14 cm., respectively. A frusto-conical tube portion with a length of 6 cm. formed the connection between the tube portions.

Physical properties of the yarn so manufactured were: the secondary swell value was 68% (i.e., the percentage 35 of water retained in centrifuged yarn that has been washed, dried and re-wet with water); the dry strength was 4.2 g./denier; the dry elongation was 28%; the double loop strength and the abrasion resistance of the threads had a high value; and the cross sections of the 40 threads showed a yarn of substantially all skin.

#### Example II

A viscose with a cellulose content of 8.3% and an alkali content of 4.6% and containing 0.2% of the organic compound with the formula,



55 was extruded through a spinneret in the usual manner into a primary spinbath having a temperature of 50° C. The viscose had a xanthate ratio of 0.42, a viscosity of 35 sec. by the falling ball test and a ripeness of 9° Hottenroth. The said spinbath contained 4.0% H2SO4, 17.5% Na2SO4 and 3.3% ZnSO4. After leaving the spinbath, the spun threads were stretched 65% in air and taken up in the conventional way at a velocity of 55 meters per minute. The yarn was then aftertreated in the usual way.

Physical properties of the yarn so manufactured were: 60 the secondary swell value was 70%; the dry elongation and wet elongation were 32 and 36 respectively; the dry strength and wet strength were 3.1 and 2.4 g./denier, respectively, with the wet strength being relatively high with regard to the dry strength; fabric made from the 65 yarn exhibited excellent laundering properties; and the



X is selected from the group consisting of COC<sub>6</sub>H<sub>4</sub>CO, C<sub>6</sub>H<sub>4</sub>CO and



and R' is selected from H, CH<sub>3</sub> and OC<sub>2</sub>H<sub>5</sub>.

References Cited in the file of this patent

UNITED STATES PATENTS

|           |            |               |
|-----------|------------|---------------|
| 1,449,380 | Callimachi | Mar. 27, 1923 |
| 2,359,749 | Collins    | Oct. 10, 1944 |

|    |           |
|----|-----------|
| 5  | 2,535,044 |
|    | 2,593,466 |
|    | 2,664,360 |
|    | 2,696,423 |
| 5  | 2,732,279 |
|    | 2,775,505 |
|    | 2,777,775 |
|    | 2,792,313 |
| 10 | 2,805,169 |
|    | 2,841,462 |
|    | 2,849,274 |
|    | 2,852,334 |
|    | 2,890,130 |

|                |                |
|----------------|----------------|
| Cox            | Dec. 26, 1950  |
| MacLaurin      | Apr. 22, 1952  |
| Charles et al. | Dec. 29, 1953  |
| Dietrich       | Dec. 7, 1954   |
| Tachikawa      | Jan. 24, 1956  |
| Pedlow         | Dec. 25, 1956  |
| Edwards        | Jan. 15, 1957  |
| Charles et al. | May 14, 1957   |
| Mitchell       | Sept. 3, 1957  |
| Lytton         | July 1, 1958   |
| Lytton         | Aug. 26, 1958  |
| Hollihan       | Sept. 16, 1958 |
| Howsmon        | June 9, 1959   |